

Dec. 25, 1956

R. G. GUENTER

2,775,200

PRIMING DEVICE

Filed Dec. 3, 1952



FIG. 1



FIG. 2



FIG. 3



FIG. 4



FIG. 5



FIG. 6

RICHARD G. GUENTER  
INVENTOR.

BY

*Ernest G. Peterson*

AGENT.

1

2,775,200

## PRIMING DEVICE

Richard G. Guenter, Lawrence, Kans., assignor to Hercules Powder Company, Wilmington, Del., a corporation of Delaware

Application December 3, 1952, Serial No. 323,856

8 Claims. (Cl. 102—27)

This invention relates to detonating means for explosive charges and in particular to detonating devices especially adapted for use in applications where relatively insensitive explosive is employed, or where advanced temperatures are encountered which render the use of conventional blasting initiators undesirable.

In recent years there has been a trend toward the use of relatively insensitive blasting agents which contain little or no nitroglycerin and depend primarily for explosive strength upon such materials as ammonium nitrate. While these blasting agents when brought to detonation are characterized by sufficient strength for most blasting operations, they are normally not detonatable by commercially available blasting caps. In fact, the test employed to determine the sensitivity characteristics of such blasting agents is usually one in which their resistance to detonation by a No. 6 or No. 8 cap is determined.

The usual methods for detonating these explosives have involved the use of separate priming cartridges of high explosive such as trinitrotoluene (TNT) which are brought to detonation by means of commercial electric blasting caps. Alternatively a highly potent booster cap is employed which contains a base charge of about 10-30 g. of pentaerythritol tetranitrate or equivalent explosive. While both of these means of initiating explosives are operable, they still necessitate the use of blasting initiators which are expensive and which are themselves considerably more sensitive to both heat and shock than the blasting agent itself. Thus, the safety for which the insensitive blasting agents were originally designed is still not always obtainable in the degree desired by the art.

Special difficulties are encountered in shooting hot holes in which the temperatures often reach a point high enough to cause premature detonation of conventional blasting caps. A means for initiating these insensitive explosives which does not require the presence of large amounts of sensitive explosive or electric blasting caps in the borehole itself is therefore greatly to be desired.

Now in accordance with the present invention, there has been developed a means for initiating insensitive blasting agents and explosives generally which does not require the presence of either highly sensitive high explosive compositions or electric initiators of any sort in the immediate vicinity of the charge to be detonated.

Generally described, the present invention is a priming device for detonatable explosive compositions which comprises a detonatable body of compacted explosive composition containing crystalline high explosive selected from the group consisting of cyclonite (RDX) and pentaerythritol tetranitrate (PETN) and at least 15% of nitrocellulose. In accordance with one embodiment of the invention, the compacted body is associated with detonative means. Preferably, the detonative means will be a detonating fuse such as Primacord (granular PETN or RDX covered with fabric or plastic) or Cor-

2

deau (granular TNT covered with thin lead tubing containing the desired number of grains of explosive per foot and will be disposed in detonating relationship with the explosive body. Preferably, the fuse will be disposed in a recess, that is, in a well or a perforation formed in the compacted body, although other suitable disposition may be employed. In applications where resistance to heat or shock is not an important factor blasting caps may be similarly employed as the detonative means. In a preferred embodiment of the invention, the compacted explosive body is formed into a axially perforated cylinder, the perforation extending through at least a major extent of the length of the cylinder. With such a structure, the detonative means employed may be disposed in or pass through the perforation.

The compacted body of explosive composition in accordance with this invention is readily detonated by detonating fuses of the desired strength, such as Primacord and Cordeau, but is highly insensitive both to shock conditions which can normally be expected during blasting operations and to ignition or detonation by temperatures usually encountered. It is usually desirable to incorporate a small amount of stabilizer for nitrocellulose, such as diphenylamine or Centralite, in the compositions from which the compacted body is formed. The amount employed is usually in the order of .2 to 1%. While this composition will normally be sufficiently water resistant for most moisture conditions encountered, it is desirable in some instances to include a non-volatile plasticizer for nitrocellulose such as diethyl phthalate, dibutyl phthalate, dimethyl phthalate, ethyl Centralite or dinitrotoluene. While varying amounts of the plasticizer may be employed, increase in plasticizer effects a corresponding decrease in sensitivity to detonation. It has further been found that nitroglycerin can be employed in amounts up to about 5% without adversely affecting the thermal stability of the overall composition. In general, it has been found that it is unnecessary to employ more than 5% of plasticizer since this amount has been found to render these compositions sufficiently resistant to water that they will shoot with 50 grain Primacord (50 gr. PETN per foot) after days of exposure to water at pressures as high as 45 p. s. When employed in hot holes, the compacted bodies primed with Primacord have been found to function properly without violent decomposition or premature explosion at temperatures of 500 to 1000° F.

The compacted bodies are preferably made in coaxially perforated cylinders by extrusion in accordance with known smokeless powder extrusion techniques. However, the compacted bodies may have any desired shape and may be molded by any desired process.

Having generally described the invention, several embodiments will be more specifically illustrated with reference to the accompanying drawings in which Fig. 1 represents a longitudinal section of a cylindrical compacted body in accordance with the invention; Fig. 2 is a sectional end view of Fig. 1; Fig. 3 is a part elevational, part sectional view of the body of Figs. 1 and 2 primed with detonating fuse; Fig. 4 is a part sectional, part elevational view of an explosive cartridge primed with the device of Fig. 3; Fig. 5 is a part sectional, part elevational view of a cylindrical compacted body primed with an electric initiator; and Fig. 6 is a side elevation of a borehole primed in accordance with the invention.

Referring now to the drawings in which like numbers represent similar parts, and particularly to Figs. 1 to 4, a cylindrical compacted body 10 of explosive composition in accordance with this invention is provided with a coaxial perforation 11. A length of detonating fuse 12 is passed through the coaxial perforation 11 of the

body 10 and is suitably secured therein. In Fig. 3, the detonating fuse is secured within the perforation by means of a knot tied in the detonating fuse which prevents its withdrawal.

In Fig. 4, a cartridge 13 of insensitive explosive is equipped with a coaxial bore 14 defined by a hollow tube 15 passing concentrically through the cartridge 13. The hollow tube is indented at 16 to provide a detent means. Concentrically perforated, compacted body of explosive in accordance with the invention is disposed in the coaxial bore 14 and is prevented from passing therethrough by the indentation 16 in the tube 15. Detonating fuse 12 passes through the compacted body 10 and extends completely through the coaxial bore 14 of the cartridge 13. The leading end of the detonating fuse 12 is passed

15 be detonated at a safe distance from the borehole 23 by means of an electric initiator.

The following examples are presented to more specifically illustrate embodiments of the invention. In the 5 table, Examples 1 to 24 illustrate different compositions for the compacted body. The water resistance of these compositions and the comparative sensitivity to detonation of wet and dry compositions are set forth. The compacted bodies tested were in the form of coaxially 10 perforated cylinders 4 inches in length and 0.67 inch in diameter. The diameter of the perforation was about 0.27 inch. These cylinders were prepared by conventional smokeless powder compounding and extrusion techniques as hereinafter described. All compositions were stabilized 15 with 0.3% of diphenylamine.

| Ex. | Explosive, Percent |      |                     |             | Primacord Sensitivity <sup>1</sup> |        |        |        |         |                                 |        |        |        |        |         |
|-----|--------------------|------|---------------------|-------------|------------------------------------|--------|--------|--------|---------|---------------------------------|--------|--------|--------|--------|---------|
|     |                    |      |                     |             | Dry                                |        |        |        |         | Wet—45 Lbs. Pressure for 5 Days |        |        |        |        |         |
|     | RDX                | PETN | NC                  | Plasticizer | 30 Gr.                             | 40 Gr. | 50 Gr. | 60 Gr. | 100 Gr. | Water Pickup, percent           | 30 Gr. | 40 Gr. | 50 Gr. | 60 Gr. | 100 Gr. |
| 80  |                    | 19.7 | 0 DEP               | S           |                                    |        |        |        |         | 12.25                           | F      | F      | PS     | PS     | S       |
| 80  |                    | 19.7 | 1 <sup>st</sup> DEP | PS          | PS                                 | S      |        |        |         | 7.90                            | F      | F      | PS     | PS     | S       |
| 80  |                    | 19.7 | 2 <sup>nd</sup> DEP | PS          | PS                                 | S      |        |        |         | 6.52                            | F      | F      | PS     | S      |         |
| 80  |                    | 19.7 | 3 <sup>rd</sup> DEP | F           | PS                                 | S      |        |        |         | 4.67                            | F      | F      | PS     | PS     | S       |
| 80  |                    | 19.7 | 4 <sup>th</sup> DEP | F           | PS                                 | S      |        |        |         | 1.50                            | F      | PS     | S      |        |         |
| 80  |                    | 19.7 | 5 <sup>th</sup> DEP | F           | PS                                 | PS     | S      |        |         | 0.74                            | F      | F      | PS     | S      |         |
| 80  |                    | 19.7 | 6 <sup>th</sup> DEP | F           | PS                                 | S      | PS     | S      |         | 0.00                            | F      | F      | PS     | S      |         |
| 80  |                    | 15.7 | 4 DEP               | F           | PS                                 | S      |        |        |         | 1.16                            | F      | PS     | PS     | PS     | S       |
| 85  |                    | 10.7 | 4 DEP               | F           | PS                                 | S      |        |        |         | 5.19                            | F      | F      | S      |        |         |
| 75  |                    | 24.7 | 0                   | PS          | S                                  |        |        |        |         | 11.87                           | F      | F      | PS     | PS     | PS      |
| 75  |                    | 20.7 | 4 DEP               | F           | PS                                 | S      |        |        |         | 1.38                            | F      | F      | PS     | S      | PS      |
| 75  |                    | 19.7 | 5 NG                | PS          | PS                                 |        |        |        |         | 0.52                            | F      | PS     | S      |        |         |
| 75  |                    | 19.7 | 5 DNT               | F           | PS                                 | S      |        |        |         | 1.29                            | F      | PS     | S      |        |         |
| 75  |                    | 19.7 | 5 TNT               | F           | PS                                 | S      |        |        |         | 1.07                            | F      | PS     | S      |        |         |
| 80  |                    | 19.7 | 0                   | S           |                                    |        |        |        |         | 8.03                            | S      |        |        |        |         |
| 80  |                    | 19.7 | 1 <sup>st</sup> DEP | S           |                                    |        |        |        |         | 9.96                            | PS     | PS     | S      |        |         |
| 80  |                    | 19.7 | 2 <sup>nd</sup> DEP | S           |                                    |        |        |        |         | 10.10                           | PS     | PS     | S      |        |         |
| 80  |                    | 19.7 | 3 <sup>rd</sup> DEP | S           |                                    |        |        |        |         | 9.77                            | PS     | PS     | S      |        |         |
| 80  |                    | 19.7 | 4 <sup>th</sup> DEP | S           |                                    |        |        |        |         | 3.88                            | PS     | S      |        |        |         |
| 80  |                    | 19.7 | 5 <sup>th</sup> DEP | S           |                                    |        |        |        |         | 1.90                            | PS     | S      |        |        |         |
| 80  |                    | 19.7 | 6 <sup>th</sup> DEP | S           |                                    |        |        |        |         | 1.57                            | S      |        |        |        |         |
| 75  |                    | 24.7 | 0                   | S           |                                    |        |        |        |         | 5.15                            | PS     | S      |        |        |         |
| 70  |                    | 29.7 | 0                   | S           |                                    |        |        |        |         | 5.09                            | F      | PS     | S      |        |         |
| 80  |                    | 16.7 | 3 DEP               | S           |                                    |        |        |        |         | 11.01                           | F      | PS     | S      |        |         |

<sup>1</sup> Tested by shooting with PETN Primacord of indicated strength.

RDX—cyclonite.

PETN—pentaerythritol tetranitrate.

NC—nitrocellulose.

DEP—diethyl phthalate.

NG—nitroglycerin.

DNT—dinitrotoluene.

TNT—trinitrotoluene.

S—shot, hole in plate.

PS—shot, dent in plate.

F—failed.

\*Plasticizer added to composition.

ough a centrally orificed wooden disk 17 which has a diameter greater than that of the tube 15. The leading end of the detonating fuse 12 is knotted to prevent its passage through the disk 17. The priming cartridge 13 may be lowered into a borehole by means of the detonating fuse 12 and the compacted priming body 10 is thus retained in position in the central portion of the cartridge 13.

In Fig. 5, a cylindrical, compacted body 18 in accordance with the invention is provided with a well 19. An electric initiator 20 is disposed in the well 19 and connected to a current source (not shown) by lead wires 21. In Fig. 6, blasting cartridges 22 are disposed in a vertical borehole 23. The lower cartridge 22 is primed in accordance with the invention by disposing a coaxially perforated cylindrical body 10 of explosive composition, as shown in Fig. 1, in the upper portion of the cartridge. A length of Primacord 12 passes laterally through the cartridge 22 and through the coaxial perforation of the compacted body 10. The Primacord 12 is then tied as shown and leads out of the borehole. The remaining cartridges are disposed on top of the lower primed cartridge. The bore hole is stemmed as at 25. The Primacord 12 may

#### Example 25

Field trials were conducted in which several boreholes 55 were loaded with commercial blasting cap insensitive blasting agent principally comprising ammonium nitrate. The temperature in these boreholes was between 400-500° F. due to underground fires. In each hole a primer cartridge was employed similar to that shown in Fig. 4. The primer 60 cartridge contained commercial blasting cap insensitive blasting agent. The compacted body was similar to that of Example 1 and contained 80% RDX, 19.7% NC, and .3% diphenylamine. A 50 grain PETN Primacord 65 was employed which was initiated at a distance from the hole by means of an electric blasting cap. After being loaded, the holes were not fired for about 20 minutes. All holes fired normally and with no indication of any decomposition of the compacted body in the primer cartridge.

From the foregoing examples, and especially from Examples 1 to 24, it will be seen that the composition of the compacted bodies may be subject to considerable variation. It has been found, however, that at least 15% of nitrocellulose must be employed in order to obtain a compacted body having the requisite physical strength and to

obtain the necessary extrusion characteristics. When less than 15% of nitrocellulose is employed, the bodies do not compact well and are crumbly.

The amount of crystalline explosive employed will depend on the degree of sensitivity required for the particular application. Due to the fact that PETN is more sensitive to detonation than RDX, less PETN than RDX need be used with a detonating fuse of a particular strength. Similarly, the amount and nature of the plasticizer may be varied to give the desired characteristics in terms of water resistance and sensitivity to heat and shock. For commercially available detonating fuse, it has been found desirable to employ at least 75% of RDX and at least 70% of PETN.

While cylindrical compacted bodies of RDX or PETN with nitrocellulose have been employed to specifically illustrate the invention, the invention is not so limited, since as previously indicated the compacted bodies may be of any desired shape.

The compacted bodies are easily produced by the usual smokeless powder process. In accordance with the preferred process, the nitrocellulose, wet with 2B alcohol, is placed in a sigma-blade mixer together with the stabilizer and plasticizer, if used, the particulate explosive, acetone, and additional 2B alcohol. The ingredients are then thoroughly mixed, preferably for about 3 hours. In accordance with the preferred procedure, the composition is then extruded through a die of the desired dimensions, the perforation being formed by a die pin of a size slightly larger than the detonating fuse to be employed. The compacted, extruded bodies are dried in air at a temperature of about 120-140° F. to effect solvent removal. Alternatively, however, the paste from the mixer may be compression molded in a suitable mold and the solvent removed by drying as before. The RDX or PETN employed should be finely divided.

From the foregoing, it will be seen that the priming devices of the invention have many advantages. Devices having high heat or shock resistance may be prepared which when detonated, are highly brisant and capable of satisfactorily initiating insensitive blasting agents or other explosive composition. While the compacted bodies may be made in any size, small, inexpensive bodies are satisfactory. These bodies are structurally self-sufficient and require no metal or plastic shells for support. What is of great importance from the standpoint of both manufacturer and user is that the compacted bodies can be easily and economically prepared by utilizing known smokeless powder extrusion techniques and equipment. Other advantages will be apparent to those skilled in the art.

While the explosive priming device of the invention will have primary utility when used with the currently popular insensitive blasting agents, the device can also be used with more sensitive explosives if desired. In like manner, although the device has special utility for shooting hot holes, its use is not so restricted. It is intended that

the scope of this invention be defined solely by the scope of the appended claims.

What I claim and desire to protect by Letters Patent is

1. As a new article of manufacture a priming device for detonating blasting charges comprising a compact explosive composition formed as a cylinder, the walls of said cylinder forming an annulus about a substantially coaxially disposed perforation extending through at least a major extent of the length of the cylinder and adapted to contain a detonating means, said explosive consisting essentially of at least 75 percent cyclonite and at least 1 percent nitrocellulose to form an independent cohesive body.

15 2. An article of claim 1 wherein said perforation extends through said cylinder.

3. An article of claim 1, wherein said detonating means is a detonating fuse disposed in at least a portion of said perforation in propagating relationship with said compacted composition.

20 4. An article of claim 1 wherein the said compacted explosive contains not in excess of about 5 percent of nonvolatile plasticizer for nitrocellulose.

5. As a new article of manufacture a priming device for detonating blasting charges comprising a compact explosive composition formed as a cylinder, the walls of said cylinder forming an annulus about a substantially coaxially disposed perforation extending through at least a major extent of the length of the cylinder and adapted to contain a detonating means, said explosive consisting essentially of at least 70 percent pentaerythritol tetrinitrate and at least 15 percent nitrocellulose to form an independent cohesive body.

6. An article of claim 5 wherein said perforation extends through said cylinder.

35 7. An article of claim 5 wherein said detonating means is a detonating fuse disposed in at least a portion of said perforation in propagating relationship with said compacted composition.

8. An article of claim 5 wherein the compacted explosive contains not in excess of about 5 percent of nonvolatile plasticizer for nitrocellulose.

#### References Cited in the file of this patent

#### UNITED STATES PATENTS

|    |           |                       |                |
|----|-----------|-----------------------|----------------|
| 45 | 58,656    | Lucas -----           | Oct. 9, 1866   |
|    | 905,336   | Lheure -----          | Dec. 1, 1901   |
|    | 2,407,595 | Williams et al. ----- | Sept. 10, 1946 |
|    | 2,425,854 | Alexander -----       | Aug. 19, 1948  |
| 50 | 2,429,246 | Traylor -----         | Oct. 21, 1949  |
|    | 2,709,407 | Lowe -----            | May 31, 1951   |

#### FOREIGN PATENTS

|    |         |                     |               |
|----|---------|---------------------|---------------|
| 55 | 20,281  | Great Britain ----- | of 1894       |
|    | 20,110  | Great Britain ----- | of 1911       |
|    | 145,791 | Great Britain ----- | Mar. 17, 1921 |
|    | 343,485 | Great Britain ----- | Feb. 16, 1931 |